

# UNITED STATES PATENT OFFICE.

HOWARD FREDERICK WEISS, OF MADISON, WISCONSIN, ASSIGNOR TO C. F. BURGESS  
LABORATORIES, A CORPORATION OF WISCONSIN.

## FIREPROOFING WOOD.

1,339,488.

Specification of Letters Patent. Patented May 11, 1920.

No Drawing.

Application filed January 23, 1919. Serial No. 272,643.

To all whom it may concern:

Be it known that I, HOWARD F. WEISS, a citizen of the United States, residing at Madison, in the county of Dane, State of Wisconsin, have invented certain new and useful Improvements in Fireproofing Wood; and I do hereby declare the following to be a full, clear, and exact description of the invention, such as will enable others skilled in the art to which it appertains to make and use the same.

This invention relates to a method of rendering wood and similar fibrous material fireproof by depositing an insoluble salt in the fibers of the material, and has for its primary object the provision of a method whereby the fireproofing operation is facilitated and rendered less expensive without detracting from the quality of the product resulting from the operation.

It has heretofore been suggested to impregnate fibrous materials with insoluble borates by first saturating the material with a soluble borate, then drying the material and finally saturating it with a soluble salt of lead. Only a relatively small amount of insoluble borate is thus precipitated in the fibers, and in order to accomplish the desired result it has been necessary to use a relatively large quantity of the chemicals employed, the greater proportion of which remains in the product, when dried, in a form ineffective to accomplish the desired result of fireproofing the material. This ineffective filling adds greatly to the weight of the product, thereby increasing the shipping charges thereon.

Furthermore, the formation in the fibers of an insoluble borate, by injecting into the wood a solution of a soluble compound of boric acid followed by a second injection of a soluble metallic salt, produces an indefinite yield of insoluble borate, which is the essential fire proofing agent in such a treatment.

I have discovered that the yield of insoluble borate may be greatly augmented by rendering the solution of soluble borate somewhat strongly alkaline preferably before it is applied to the fibrous material. I have also discovered that it is unnecessary to thoroughly dry the material between the

steps of saturating with the soluble borate and with the precipitating agent. The method is particularly applicable to the fireproofing of shingles, clapboards and the like building material, exposed to the weather.

By following the method as hereinafter described, the yield of insoluble borate is greatly increased with a given quantity of chemicals and accordingly the amount of chemicals employed may be reduced to a considerable extent, thus rendering the process less expensive and also lowering the shipping weight of the product.

In carrying out the method I preferably treat the material in a closed cylinder or other suitable apparatus to which a vacuum or pressure may be applied at will. The material in such apparatus is first subjected to a vacuum to withdraw the air therefrom and is then, without breaking the vacuum, treated with a solution containing preferably 6% or over of a soluble borate to which a proportion of a suitable alkali, for example sodium hydrate, sodium carbonate, potassium hydrate, or potassium carbonate has been added. The exact proportions of the borate and alkali may be varied, suitable proportions being five parts of soluble borate and one part of alkali in the case of magnesium sulfate. I then apply a pressure of about 75 pounds per square inch to the solution, thereby forcing it in the fibers of the material until the latter is partially or thoroughly saturated. The treatment may be continued for varying periods, for example, 240 minutes, the solution being preferably maintained at a temperature in the neighborhood of 90 degrees C. All these factors of treatment vary, dependent upon the character of the material being treated. As soon as the material is saturated to a sufficient extent the solution is removed and the material is again subjected to a vacuum. Without breaking the vacuum I admit the precipitating reagent, which may be a solution of any soluble salt capable of reacting with the soluble borate to precipitate an insoluble borate in the fibers of the material. Various reagents may be employed, as for example, zinc chlorid, magnesium sulfate, and ferric and ferrous sulfate. I prefer

2  
magnesium sulfate because of its cheapness and the excellent results that can be secured with it. The precipitating reagent is subjected to a pressure of about 100-150 pounds per square inch and the treatment is continued for a suitable period, for example, 240 minutes, the solution being maintained at a temperature in the neighborhood of 90 degrees C. These factors are determined by 5 the particular character of the material being treated. When the treatment has been completed the excess solution is withdrawn and the material is removed.

As will be readily understood, the method 10 as hereinbefore defined is substantially continuous until the completion thereof, there being no necessity for intermediate drying of the material. I find that the efficiency of the method, owing to the presence 15 of the excess of alkali, is increased at least 10% in the precipitation of insoluble borates over the best results obtainable where a soluble borate alone is used without the alkali. The final product, owing to the 20 employment of smaller quantities of chemicals, contains a lower proportion of ineffective soluble salts. If desired, the soluble salts present may be removed by washing the treated material with water after the 25 precipitating reagent has been used. The washing may be accomplished in the treating cylinder or any other suitable apparatus, as desired. The washing has an additional beneficial effect, aside from the removal 30 of the insoluble salts which reduces the weight of the product, in that it improves the appearance of the product and reduces its tendency to corrode nails and similar metal articles with which it comes 35 in contact, the soluble chlorides and sulfates 40 which have a deteriorating action on metals being removed by the washing.

While I have described the method as carried out in an apparatus in which a vacuum 45 and pressure may be employed, it is to be understood that my invention is in no way limited to any particular type of apparatus, it being possible to secure entirely satisfactory results by saturating the material with 50 the respective solutions in open tanks and without employing either vacuum or pressure. The method is of course facilitated and the time required is considerably decreased by employing a vacuum and pressure 55 sure where apparatus for this purpose is readily available.

It is to be understood that various changes may be made in the details of the method as hereinbefore described and that 60 various equivalent chemicals may be substituted within the scope of the appended claims, without departing from the spirit of the invention or sacrificing any of its material advantages.

I claim:

1. A method of fire proofing fibrous material which comprises impregnating the material with an aqueous borate solution containing an excess of alkali, and then impregnating the material with a solution 70 of a reagent capable of reacting with the first solution to precipitate an insoluble borate in said material.

2. A method of fire proofing fibrous material which comprises impregnating the 75 material with an aqueous borate solution containing an excess of sodium hydrate, and then impregnating the material with a solution of a metal salt capable of reacting with the first solution to precipitate an in- 80 soluble borate in said material.

3. A method of fire proofing fibrous material which comprises impregnating the material with an aqueous borate solution containing an excess of alkali, and then impregnating the material with a solution of magnesium salt capable of reacting with the first solution to precipitate an insoluble borate in said material. 85

4. A method of fireproofing fibrous ma- 90 terial which comprises impregnating the material with a solution of a soluble compound of boric acid and a soluble alkali, withdrawing the unabsorbed solution and impregnating the material with a reagent 95 capable of reacting with said solution to precipitate an insoluble compound of boric acid in said material.

5. A method of fireproofing fibrous ma- 100 terial which comprises impregnating the material under pressure with a solution of a soluble compound of boric acid and a soluble alkali, withdrawing the unabsorbed solution and impregnating the material 105 under pressure with a reagent capable of reacting with said solution to precipitate an insoluble compound of boric acid in said material.

6. A method of fireproofing fibrous ma- 110 terial which comprises impregnating the material with a solution of a soluble compound of boric acid and subjecting the ma- 115 terial while still in a moist condition to the action of a reagent capable of reacting with the soluble boric acid compound to precipi- 118 tate an insoluble compound thereof.

7. A method of fireproofing fibrous ma- 120 terial which comprises subjecting the ma- 125 terial under pressure to a solution containing a soluble compound of boric acid, re- moving the excess of such solution, and subjecting the material under pressure and while still in a moist condition to the action of a reagent capable of reacting with the soluble boric acid compound to precipitate 128 an insoluble compound thereof.

8. A method of fireproofing fibrous ma- 130 terial which comprises subjecting the ma-

terial to a vacuum, impregnating the material under pressure with a solution containing a soluble compound of boric acid, withdrawing the excess of such solution and  
5 again subjecting the material to a vacuum, causing a reagent capable of reacting with said solution to form an insoluble com-

pound of boric acid, to impregnate the material under pressure while the material is still in a moist condition, and finally removing the excess of said reagent. 10

In testimony whereof I affix my signature.

HOWARD FREDERICK WEISS.